

# UNITED STATES PATENT OFFICE.

HUGH RODMAN, OF PITTSBURG, PENNSYLVANIA.

## CARBONIZING OR CASE-HARDENING LOW-CARBON STEEL.

949,447.

Specification of Letters Patent. Patented Feb. 15, 1910.

No Drawing.

Application filed May 15, 1909. Serial No. 496,272.

*To all whom it may concern:*

Be it known that I, HUGH RODMAN, a citizen of the United States, and a resident of Pittsburg, in the county of Allegheny and State of Pennsylvania, have made a new and useful Invention in Carbonizing or Case-Hardening Low-Carbon Steel, of which the following is a specification.

This invention relates to the art of carbonizing or case-hardening low carbon steel or iron and to cementing material for use therein.

I have found that many coals, especially the soft coals, by which I mean bituminous coal, cannel coal, lignites and peats, develop active cementing properties when mixed with various compounds of the fixed bases for example Ca, Ba, Na, K and the like and produce cementing material which will not

20 may the surface of the metal parts treated.

I have found that by mixing bituminous coal, such as is generally found in the Pittsburg district, Colorado lignites, cannel coals and peats from various localities, with, say, 25 10% of powdered lime and 5% of soda-ash, or, say, 25% of barium carbonate, I produce an excellent cementing material. In order to maintain a thorough admixture of the materials, which are liable to more or less 30 separate on account of the different densities of the constituents, I find it preferable, but not necessary, to mix with such materials about 5% of oil, such as crude petroleum.

35 It is necessary that the cementing material should not pit or mar the surface of the metal parts treated and I have found

that in order to preserve a good surface on the metal parts it is essential that in selecting the energizing materials those evolving 40 harmful substances such as fluorin must be avoided.

Having thus described my invention, what I claim is:

1. Cementing or case hardening material 45 containing soft coal and a compound of a fixed base.

2. Cementing or case hardening material containing soft coal and lime.

3. Cementing or case-hardening material 50 containing soft coal, lime and soda-ash.

4. Cementing material containing coal of the lignite or peat series and a compound of a fixed base.

5. Cementing or case-hardening material 55 containing coal of the lignite or peat series and lime.

6. Cementing material containing coal of the lignite or peat series, lime and soda-ash.

7. Cementing or case-hardening material 60 containing coal and lime.

8. Cementing or case-hardening material containing coal, lime and soda-ash.

9. Cementing or case hardening material containing soft coal and soda ash.

10. Cementing or case hardening material 65 containing coal and soda ash.

In testimony whereof, I have hereunto subscribed my name this 12th day of May, 1909.

HUGH RODMAN.

Witnesses:

C. W. McGHEE,  
GEO. C. WALKER.